

1

2,997,507

METALLIC CORROSION INHIBITION OF POLY-HALOGENATED HYDROCARBONS WITH PROPARGYLDIISOPROPYLAMINE

Roger F. Monroe and Donald E. Rapp, Midland, Mich., assignors to The Dow Chemical Company, Midland, Mich., a corporation of Delaware

No Drawing. Filed Dec. 3, 1958, Ser. No. 777,820

8 Claims. (Cl. 260—652.5)

The present invention relates to anticorrosion agents and antioxidants, and is more particularly concerned with prevention of corrosion and oxidation of and in, chlorinated aliphatic hydrocarbon solvents to obtain solvent compositions having improved stability at elevated temperatures and to chlorinated aliphatic hydrocarbon solvents containing an amine having the general formula:



wherein each R represents a lower aliphatic hydrocarbon radical, at least one of which contains ethylenic or acetylenic unsaturation, the total number of carbon atoms in the three R's being from 4 to 10, inclusive.

It is well known that chlorinated aliphatic hydrocarbon solvents are unstable under heat, light, air and metal contact. The field wherein all of these conditions are found is the art of vapor degreasing. In the art of degreasing metals, for example, the chlorinated aliphatic hydrocarbons have been employed to the almost total exclusion of other solvents. These compounds, desirable because of their substantial high solvent action under the conditions of use and relative freeness from fire hazards, have major drawbacks, such as their instability under acid conditions. Mineral acids cause the degradation of the chlorinated hydrocarbon solvents, the degradation products including, in many instances, HCl. Thus, the degradation progresses in a somewhat chain-like manner to increase the acidity of the solution and thus catalyze further degradation. Further, long-chain fatty acids commonly introduced into the system by buffering compounds, cutting oils, etc., deplete the usual basic (amine) acid-acceptors thus permitting the mineral acids as formed to cause further degradation.

It is, therefore, an object of the present invention to provide an additive which when present in minor quantities in chlorinated hydrocarbon solvents will prevent the degradation of the solvent. A further object is to provide an additive which will prevent the corrosion of metal in contact with the solvents, thereby prolonging the useful life of such solvents and the metal in contact therewith. Another object is to provide an additive which in minor amounts will remain effective in the chlorinated hydrocarbon solvents in both the liquid and vapor phases. A still further object is to provide an ingredient which will prevent corrosion and oxidation under acid conditions and which will not be depleted by the acid conditions. These and other objects will become apparent to those skilled in the art from the following specification and claims.

It has now been found that substantial inhibition of the build-up of acid, the prevention of corrosion and oxidation, and the protection of the usual stabilizers em-

2

ployed in chlorinated hydrocarbon solvents is achieved when an amine having the formula



wherein each R has the aforesaid significance, is added to chlorinated hydrocarbon solvent compositions. Further commercial solvents containing the usual additives, such as, diisopropylamine, butylene oxide, isopropyl acetate and 2,4,4-trimethyl-2-pentene are effectively protected from acid buildup oxidation, corrosion and depletion of the inhibitors. Good results are obtained when the amine is employed in amounts of from 50 to 5,000 parts by weight per million parts of chlorinated hydrocarbon. An advantage of the amines of the present invention is that they are not immobilized or bound in the liquid phase but are found in effective concentration in both the liquid and vapor phase. Thus, corrosion is minimized in both phases, yet the compound is not immobilized as are the usual hydrogen chloride acceptors such as the saturated amines. The inhibitor of the present invention prevents the oxidation of the solvent in the presence of air and/or light, thus preventing the degradation of the solvent. The additives of the present invention are found to be effective as antioxidants even after the development of more than stoichiometric quantities of HCl or other acids in the system.

Compounds which can be employed in the practice of the invention and falling within the general formula:



are 3-dimethylamino-3-methyl-1-butyne, 3-dimethylamino-1-pentyne, allyldiisopropyl amine, triallylamine, diallylpropylamine, allyldiethylamine, propargyldiisopropylamine, and the like.

The following examples are illustrative of the present invention but are to be construed as limiting the same.

#### ACCELERATED OXIDATION TEST (MIL-T 7003)

A trichloroethylene formulation is heated at the reflux temperature for 48 hours in the presence of incandescent light, oxygen and iron. The formulation must not develop more than 200 parts per million (p.p.m.) of acid as HCl to be acceptable as a commercial degreasing solvent. A trichloroethylene formulation containing 3,000 p.p.m. of butylene oxide, 2,500 p.p.m. of isopropyl acetate, and 1,500 p.p.m. of 2,4,4-trimethyl-2-pentene was employed as a typical commercial solvent and hereinafter is referred to as Formulation A.

#### ACID ACCEPTANCE DETERMINATION

A 20 ml. sample of a typical commercial solvent formulation (as above described) is refluxed for 5 minutes with an excess of alcoholic HCl over that required to react with the inhibitor. Thereafter, 25 ml. of water is added containing phenolphthalein. The formulation is back-titrated with standard NaOH solution. Percent acid acceptance is calculated as percent NaOH. This determination is run before and after the accelerated oxidation test on samples drawn from solvents used in that test.

## Examples 1 through 5

The above tests were carried out with solvent Formulation A, as set forth above, both alone and also with the indicated additives. The results tabulated below are determined before and after the accelerated oxidation test.

| Example No. | Formulation                                             | Accelerated Oxidation Test Acid in p.p.m. |          | Acid Acceptance Determination as Percent NaOH |                 |
|-------------|---------------------------------------------------------|-------------------------------------------|----------|-----------------------------------------------|-----------------|
|             |                                                         | Before                                    | After    | Before Accelerated                            | After Oxidation |
| 1           | A                                                       | 8                                         | over 200 | 0.150                                         | 0               |
| 2           | A+3-dimethylamino-3-methyl-1-butyne (500 p.p.m.)        | 6                                         | 3        | 0.147                                         | 0.119           |
| 3           | A+Allyldiisopropylamine (500 p.p.m.)                    | 53                                        | 11       | 0.196                                         | 0.100           |
| 4           | A+propargyldiisopropylamine (500 p.p.m.)                | 16                                        | 14       |                                               |                 |
| 5           | Trichloroethylene+propargyldiisopropylamine (52 p.p.m.) | 22                                        | 0        |                                               |                 |

## Example 6

In the manner of Examples 1-4, employing like solvent compositions except that the initial acid content was higher, the following results were obtained:

|                                                            |  | P.p.m. Acid as HCl |          |
|------------------------------------------------------------|--|--------------------|----------|
|                                                            |  | Before             | After    |
| Trichloroethylene (A)                                      |  | 60                 | over 200 |
| Trichloroethylene (A)+500 p.p.m. propargyldiisopropylamine |  | 50                 | 6        |

## Example 7

A 50 ml. portion of the solvent composition of A containing 500 p.p.m. propargyldiisopropylamine was refluxed for 7 days with a 2½ inch x ½ inch metal test coupon of one of the below-listed metals. The test was run simultaneously with a solvent mixture of trichloroethylene and 52 p.p.m. of propargyldiisopropylamine only. The results are tabulated below:

|                                                       | Mils Penetration per Year |       |      |      |      |
|-------------------------------------------------------|---------------------------|-------|------|------|------|
|                                                       | Al                        | Brass | Cu   | Fe   | Zn   |
| A+500 p.p.m. propargyldiisopropylamine                | 0.00                      | 0.03  | 0.01 | 0.00 | 0.70 |
| Trichloroethylene+52 p.p.m. propargyldiisopropylamine | 0.51                      |       |      | 0.78 | 0.24 |

## Example 8

A laboratory degreaser was run with a trichloroethylene solvent A+500 p.p.m. of propargyldiisopropylamine to which had been added 30 percent by volume of mineral oil for approximately 28 days with test plates of zinc, brass, iron and aluminum in the cooling coils, warm dip, and boiling sump. The solvent was found to have an acid acceptance equivalent to 0.50 percent of sodium hydroxide in the warm dip at the end of this run and the corrosion rate of the plates at the various points was negligible.

## Example 9

Trichloroethylene containing 3000 parts per million, by weight of butylene oxide 2500 p.p.m. of ethyl acetate, 1500 p.p.m. of trimethylpentene and 500 p.p.m. of an amine was treated with 10 percent by weight of oleic acid. The solvent was distilled off and an accelerated oxidation test was run as disclosed above. The results of such tests are set forth below:

|                            | Acidity in p.p.m. before and after Accelerated Oxidation Test |            |
|----------------------------|---------------------------------------------------------------|------------|
|                            | Before                                                        | After      |
| Propargyl diisopropylamine | 23                                                            | 165        |
| Allyl diisopropylamine     | 23                                                            | 50         |
| Ethyl diisopropylamine     | 23                                                            | 1 over 200 |

10 1 Titration stopped at 200.

15 It is thus apparent that halogenated hydrocarbon solvents may be stabilized against acid condition by employing the compounds of the present invention in the manner hereinbefore described. Solvents may be stabilized, in addition to trichloroethylene are, for example, carbon tetrachloride, ethylene dichloride, methyl chloroform, perchloroethylene and the like.

20 The compounds of the present invention have been shown to exhibit anticorrosion properties in both the vapor and liquid phases of the degreasing operation. Further, these compounds are recoverable with the solvent in clean-up operations.

25 This application is a continuation in part of our co-pending applications Serial Nos. 713,522 and 713,523 both filed February 6, 1958, both now abandoned.

We claim:

1. A stabilized halogenated aliphatic hydrocarbon solvent comprising from 50 to 5,000 parts by weight of a compound having the formula



35 wherein the three R's each represent a lower aliphatic hydrocarbon radical, at least one of them being unsaturated, the total number of carbon atoms in the three being from 4 to 10 inclusive, per million parts by weight of solvent.

2. A solvent composition as set forth in claim 1 wherein the compound is 3-dimethylamino-3-methyl-1-butyne.

3. A solvent solution as set forth in claim 1 wherein the compound is allyldiisopropylamine.

4. A solvent solution as set forth in claim 1 wherein the compound is propargyldiisopropylamine.

45 5. A stabilized trichloroethylene solvent comprising from 50 to 5,000 parts by weight of a compound having the formula



50 wherein the three R's each represent a lower aliphatic hydrocarbon radical, at least one of them being unsaturated, the total number of carbon atoms in the three being from 4 to 10 inclusive, per million parts by weight of solvent.

6. A solvent composition comprising trichloroethylene and from 50 to 5,000 parts by weight of 3-dimethylamino-3-methyl-1-butyne.

7. A solvent solution comprising trichloroethylene and from 50 to 5,000 parts by weight of allyldiisopropylamine.

65 8. A solvent solution comprising trichloroethylene and from 50 to 5,000 parts by weight of propargyldiisopropylamine.

## References Cited in the file of this patent

## UNITED STATES PATENTS

- 70 2,043,257 Missbach \_\_\_\_\_ June 9, 1936  
 2,160,944 Coleman et al. \_\_\_\_\_ June 6, 1939  
 2,476,554 Lincoln et al. \_\_\_\_\_ July 10, 1949  
 2,543,575 Harvey et al. \_\_\_\_\_ Feb. 27, 1951  
 75 2,781,406 Dial \_\_\_\_\_ Feb. 12, 1957